# EUROPEAN PATENT APPLICATION

(11) **EP 0 304 405 A1**
(43) Date of publication of application: **22.02.1989**
(21) Application number: 88830263.5
(22) Date of filing: 21.06.1988
(51) Int. Cl.: E01F 9/08

(54) **Prefabricated temporary use signaletics strip**

(30) Priority: 25.06.1987 IT 2106087
(71) Applicant: SNOLINE S.p.A., I-20098 San Giuliano Milanese Milano (IT)
(72) Inventor: Mueller, Franz, I-20098 San Giuliano Milanese (Milano) (IT); Robicci, Pierluigi, I-20098 San Giuliano Milanese (Milano) (IT)
(74) Representative: Cicogna, Franco

(57) **Abstract**

The removable marking tape (1) comprises a resilient pigmented base layer (2) consisting of non-cured elastomeric materials, into which base layer a net or fabric type reinforcement layer (7) is at least partially embedded. Reflecting glass particles (3) are rolled into the top surface of the base layer (2), and further reflecting glass as well as anti-skid particles (6) are distributed onto a film (5) of acrylic emulsion applied to said top surface. An adhesive layer (10) based on a polyisobutylene-butyl solution is provided on the bottom surface of the base layer (2).

## Description

### BACKGROUND OF THE INVENTION

The present invention relates to a prefabricated temporary use signaletics strip or band.

As is known,a presently very important need is that of suitably signalling diversions of road traffic from a road and the like.

This need both relates to maintenance works and accident situations in which the vehicle traffic is to be routed to alternative roads.

In order to provide safe conditions,mainly under high traffic and speed conditions,the diversion must be properly signalled and must be clearly visible both during the day and during the night.

After having performed the maintenance works,or removed the vehicle involved in an accident,the signaletics elements must be removed in an easy and quick way without damaging,for example,the road surface,to be replaced by a new permanent signaletics.

Known solutions generally use painting materials of the type of those used for permanent signaletics which,in addition to requiring skilled operators,have a generally insufficient duration.

Prefabricated signalling strips are also known which comprise a soft aluminium base the top face of which is covered by a painted signalling coating therein there are embedded reflecting glass particles.

These known signaletics strips,however,are very expensive and have a poor mechanical resistance,thereby they can be hardly removed from the road surface in the case in which they are well adhered to said road surface.

Moreover these known strips are not able of masking existing signaletics marks and because of wear they acquire a mirror like surface which is very dangerous for the traffic.

### SUMMARY OF THE INVENTION

Accordingly,the main object of the present invention is to provide a prefabricated signaletics strip able of overcoming the above mentioned drawbacks,that is having a suitable mechanical resistance and adapted to be easily deformed so as to fit the uneven contour of the road surface.

Another object of the present invention is to provide such a signaletics temporary strip which is able of absorbing the power transmitted by the vehicle wheels and dissipating it resiliently.

Another object of the present invention is to provide such a signaletics temporary strip which can be colored in different colors,as well as reflective colors,and which,moreover has antiwear properties and a long duration.

Yet another object of the present invention is to provide such a temporary signaletics strip which can be applied on a road surface in an easy and quick way and by simple apparatus and not skilled labour.

Yet another object of the present invention is to provide such a signaletics temporary strip which can be made starting from easily available materials and which,moreover,is very advantageous from a mere economic standpoint.

According to one aspect of the present invention,the above mentioned objects,as well as yet other objects,which will become more apparent hereinafter,are achieved by a temporary use prefabricated signaletics strips or band characterized in that it comprises a pigmented resilient plastics base layer thereto a reinforcement layer is coupled which is at least partially embedded in said base layer.

### BRIEF DESCRIPTION OF THE DRAWINGS

Further characteristics and advantages of the temporary use signaletics strips according to the invention will become more apparent hereinafter from the following detailed description of a preferred embodiment thereof,which is illustrated,by way of an indicative but not limitative example,in the figures of the accompanying drawings,where:
figure 1 is a cross-sectional view of the signaletics strip according to the present invention,showing in detail its forming layers;
figure 2 is an exploded bottom view of the strips according to the invention;
   and
figure 3 shows schematically a possible method for applying the strips according to the invention to a road surface.

### DESCRIPTION OF THE PREFERRED EMBODIMENT

With reference to the figures of the accompanying drawings, the temporary use prefabricated signaletics strips according to the present invention,which is overally indicated at the reference number 1,comprises a base layer 2 made of not cured resilient materials,for example of the acrylonitrilebutadiene type or of the butadiene-styrene,polychloro prene,ethylene-propylene,chlorosulphonated polyethylene,chlorurated polyethylene type,with the addition of suitable plasticizing materials such as chloroparaffines,cumarone resins,polyvinyl chloride,EVA with pigments and fillers.

More specifically,the base material or layer is formed in sheet shape by means of a calendering method so as to provide said base layer with easy deformation properties to easily fit the road surface and easily absorb the power transmitted by the wheels of the vehicles to quickly resiliently dissipate it,in such a way as not to cause said base layer from detaching from the road surface or ground.

Preferably,the thickness of the base layer is of substantially 0.5 mm and it is colored by using conventional colours,such as yellow and white pigments,depending on the rules of the several countries,by using titanium bioxide or lead chromate,or black and grey pigments,by using carbon black for example for masking previous signaletics marks.

In order to provide the strip with a high reflecting power,in the base layer glass particles or beads are embedded,the index of refraction of which is of 1.5 or,preferably,at least 1.9.

These glass particles or beads,which are indicated at 3 in the drawing,are embedded in said base layer by means of a hot rolling and will be preferably treated by comositions,such as xylanes,titanates,bifunctional epoxydic resins and the like able of binding the polymeric materials to improve the binding of the glass beads thereto.

In order to further improve visibility,a further surface glass bead layer can be provided which is anchored by means of a polymeric film 5 applied in a liquid condition on the top surface of the sheet and then dried.

This film,having a suitable thickness,corresponding to about a half of the diameter of the glass beads,preferably consists of a pigmented acrylic emulsion having a high binding property for the polymeric material and the glass material and good antiwear characteristics.

Above the mentioned film 5,before drying it,glass beads or particles 6 are distributed, as well as high friction materials such as sand,quartz and the like in order to provide the desired antislipping characteristics.

In order to provide the strip whith the desired mechanical resistance characteristics and to easily remove the strip after its use,for example for a period of 3-6 months,a reinforcement layer is further provided wich consists of a net 7 which is applied to the base layer immediately after the calendering step,by means of a hot rolling step.

This reinforcement layer can consist of a metal or plastics net or of a so called cord type of fabric.

This net,preferably of a nylon or polyester material,has a square or rectangular mesh,the greater side whereof extending longitudinally of the strip.

The mesh smaller side has preferably a size not greater than 6 mm and a denier not less than 70.

The net is partially embedded in tha base layer and,owing to the indicated width of the net meshes,it does not alter the properties of the strips to fit the ground.

On the bottom face of the base layer,reinforced by the disclosed net,a suitable adhesive layer can be applied by rolling,said adhesive layer being indicated at 10,preferably of the type based on a butyl-polyiso butylene solution,coated on a siliconized paper. This adhesive can be protected by a plastics siliconized liner 11,or left in a free condition,in which case the top acrylic layer supporting the glass beads may contain antiadhesive aids,such as silicones or fluorine derivatives.

From the above disclosure it should be apparent that the strip according to the invention can be easily applied to the road surface simply by pressing said strip on said road surface.The strip,moreover,can be easily removed from the road surface after the provided period of use.

While the invention has been disclosed and illustrated with reference to a preferred embodiment thereof,it should be apparent that the disclosed embodiment is susceptible to several modifications and variations all of which will come within the scope and spirit of the appended claims.

## Claims

1- A temporary use signaletics strips,of the prefabricated type,characterized in that said strip comprises a pigmented resilient plastics layer thereto a reinforcement layer is coupled,said reinforcement layer being at least partially embedded in said base layer.

2- A strip according to the preceding claim,characterized in that said base layer consists of not cured elastomeric materials,based on acrylonitrile-butadiene.

3- A strip according to claim 2,characterized in that said not cured elastomeric materials comprise butadienestyrene,polychloroprene,ethylene-propylene,chlorosulponated polyethylene,chlorurated polyethylene, with the addition of plasticizing materials such as chloroparaffines,cumarone resins,polyvinylchloride,EVA and with pigments and fillers.

4- A strip according to claim 1 further comprising on the top face of said base layer glass beads having a refraction index greater than 1.5.

5- A strip according to claim 4,characterized in that said glass beads are treated by compositions of the type of xylanes,titanates,bifunctional epoxydic resins adapted to provide binding sites with the polymeric material forming said base layer.

6- A strip according to claim 1,characterized in that said strip comprises,on the top face of said base layer,a polymeric film applied in a liquid status,consisting of a pigmented acrylic water emulsion,to said polymeric film glass beads and high friction coefficient materials being applied before drying.

7- A strip according to claim 1, characterized in that said reinforcement layer consists of a plastics,metal or cord fabric net.

8- A strip according to claim 7,characterized in that said net has square or rectangular meshes,with the greater side extending longitudinally of said strip and the smaller side having a size less than 6 mm,the denier being substantially of 70.

10- A strip according to claim 1,characterized in that said strip comprises,on the bottom face of said base layer,an adhesive layer based on polyisobutylenebutyl solutions.

11- A strip according to claim 1,characterized in that said strip comprises,on the bottom surface of said adhesive layer,a siliconized plastified liner.
